

# United States Patent

[11] 3,634,147

[72] Inventors **Lawrence E. Helwig**  
Hampton Township, Allegheny County;  
Leon L. Lewis, Butler, both of Pa.  
[21] Appl. No. **878,548**  
[22] Filed **Nov. 20, 1969**  
[45] Patented **Jan. 11, 1972**  
[73] Assignee **United States Steel Corporation**

FOREIGN PATENTS  
733,912 7/1955 Great Britain..... 148/6.3  
OTHER REFERENCES  
Tenhaven, Chem. Abs. 70:5568n, Jan. 12, 1970  
Primary Examiner—Ralph S. Kendall  
Attorney—Forest C. Sexton

[54] **CORROSION RESISTANT TIN-FREE STEEL AND  
METHOD FOR PRODUCING SAME**  
10 Claims, No Drawings  
[52] U.S. Cl..... **148/6.35,**  
29/195, 29/196.6, 117/107, 148/6.3  
[51] Int. Cl..... **C23f 7/04**  
[50] Field of Search..... **148/6.3,  
6.35; 117/107, 107.2; 29/195, 196.6**  
[56] **References Cited**  
UNITED STATES PATENTS  
3,480,483 11/1969 Wilkinson ..... 148/6.3

**ABSTRACT:** A superior corrosion-resistant tin-free steel is produced by vacuum depositing high-purity metallic chromium onto a thoroughly cleaned steel surface at a temperature within the range 500°-1,000° F., and thereafter, before the coated steel is cooled, exposing the freshly deposited coating to an oxidizing atmosphere while the steel is at a temperature of 600° to 1,000° F. The resulting vigorous high-temperature oxidation of exposed steel at cracks and pores to magnetite produces a continuous pore-free and crack-free coating which is lustrous and metallic in appearance and provides exceptional resistance to corrosion.

CORROSION RESISTANT TIN-FREE STEEL AND  
METHOD FOR PRODUCING SAME

## BACKGROUND OF THE INVENTION

The so-called "tin-free" steels, i.e., plated sheet steel substitutes for tinplate having protective coatings other than tin are well known in the art and are becoming of increasing significance in the container and canning industries. Commercial tin-free steels are usually produced by electroplating a thin layer of chromium onto the steel surface and subsequently or simultaneously forming a passive oxide or conversion coating over the chromium surface. Although metallic chromium by itself is extremely resistant to corrosion, deposited coatings are usually porous and cracked. Hence, the oxide coating is essential to seal the cracks and pores to protect the steel substrate. Crack-free chromium coatings are known in the art, but the plating conditions for producing such crack-free coatings are so inefficient that commercial adaption thereof is not practical.

Although such plating and oxidation processes as described above do provide some degree protective coatings, the processes are somewhat inefficient and not readily adapted to high-speed operation typical of tinplate production. In addition, the prior art electroplated and oxidized or converted coatings frequently have a tendency to turn brown, and are not usually completely free of cracks because the coatings may crack upon cooling after the passivation treatment.

Vacuum deposition of chromium is another well-known plating procedure which produces a good adherent and lustrous coating. Until recently, however, vacuum-deposited chromium coatings have been used almost exclusively for decorative applications rather than corrosion protection because the vapor-deposited coatings are too porous and discontinuous to protect against corrosion, even when oxidized or converted by conventional procedures. When corrosion resistance is required, vacuum-deposited chromium coatings are either deposited on a lacquered steel or are subsequently protected by a lacquer coating. Recently, vacuum-deposited chromium coatings have been used for protective applications on some steels. To be substantially continuous, and at least in part protective, such coatings must be rather thick, usually 500 microinches or more. Even when very thick, however, such chromium coatings exhibit some discontinuity and fine cracks which substantially lessen corrosion protection from more ideal values.

## SUMMARY OF THE INVENTION

We have discovered that a very thin vacuum-deposited high-purity chromium coating on a clean steel substrate, which is typically very porous and discontinuous, can be made continuous, pore-free and crack-free, providing superior corrosion protection, if the coating is quickly and vigorously oxidized at elevated temperatures immediately after deposition before any other surface oxidation or passivation reactions can occur.

It is, therefore, an object of this invention to provide a process for producing corrosion-resistant steel products, particularly tinplate substitutes, having a thin protective coating of chromium with the pores and cracks therein sealed with a corrosion-resistant oxide.

It is another object of this invention to provide a process for producing tin-free sheet steels having an adherent lustrous coating which will not brown or discolor and is readily adapted to high-speed processing equipment.

It is a further object of this invention to provide a method for improving the corrosion resistance of a steel having a thin porous and discontinuous vacuum-deposited chromium coating.

It is still another object of this invention to provide a new and improved corrosion-resistant sheet steel suitable as a substitute for tinplate.

## DESCRIPTION OF THE PREFERRED EMBODIMENT

Although any steel may be coated by the process of this invention, the process will find particular utility in the manufacture of corrosion-resistant tin-free sheet products.

Although the vacuum deposition of chromium in accordance with this invention is performed by well-known prior art techniques, it is essential that contamination of the steel surface and chromium coating be minimized. Simply stated, 10 the steel, after an essential thorough surface cleaning, is heated in a high vacuum thereby degassing the steel, and while heated under the high vacuum, the steel is exposed to high-purity chromium vapors which condense on the steel surface.

In preparing a steel strip for vacuum deposition, it is essential 15 that a good cleaning procedure be used to assure that substantially all surface oxides and oils are removed. We prefer to clean the strip with a short wash in a chelated alkaline solution followed by a one second dip in a 5 percent citric acid pickling 20 solution at 150° F. As an alternative, we have used an extended one minute cathodic cleaning procedure in a chelated 6 percent alkaline solution at 180° F. and a current density of 65 a.s.f. After pickling by any process, the sheet should of course be rinsed, preferably with alcohol or inhibited water to minimize reoxidation. After the strip is cleaned, other forms of 25 reoxidation or surface contaminations should be avoided. It is, therefore, preferable that vacuum depositing follow the cleaning procedure as soon as possible.

To commence vacuum deposition, the steel strip is heated 30 to a temperature within the range 500°-1,000° F., and preferably 600° to 800° F., in a vacuum of less than  $5 \times 10^{-4}$  torr, and preferably less than  $1 \times 10^{-4}$  torr, and preferably less than  $1 \times 10^{-4}$  torr. Heating the steel to the desired temperature under vacuum will be sufficient to effect suitable degassing 35 thereof, and hence no dwell time is required. After the desired temperature is reached, the strip is exposed to high-purity chromium vapors or a vapor beam in accordance with any of the various prior art practices. For example, elemental or alloyed chromium in solid form will sublime upon heating with 40 an electron beam or resistance heated conical tungsten wire basket. The chromium vapors thus formed will condense on the cooler steel surface.

The vacuum-deposited chromium coating should be applied 45 at a preferred thickness of from 1 to 3 microinches. Although any thickness within the range 0.2 to 20 microinches or more will provide some benefit, the 1 to 3-microinch coatings are optimal. Coatings less than about 1 microinch are somewhat inferior in the final corrosion protection, while coatings thicker than about 3 microinches utilize excessive chromium 50 without improvement.

As would be expected, the exceptionally thin coatings produced as described above would be quite porous and somewhat discontinuous, especially on unpolished surfaces such as that of the cold-rolled steel strip. By itself therefore, the vacuum-deposited chromium coating would afford little protection against corrosion. The crux of this invention, therefore, resides in the following oxidation step whereby the thin vacuum-deposited chromium coating is made continuous and protective to the steel substrate. That is, after the desired 55 vacuum deposition of chromium is complete, the freshly coated strip, while still at elevated temperatures of 600° to 1,000° F. is quickly exposed to an oxidizing atmosphere such as air, as for example by exiting the strip from the vacuum chamber. The hot steel exposed at cracks and pores is thereby vigorously and rapidly oxidized to a more complete state of oxidation than is possible at lower temperatures. Upon cooling, the oxidized chromium coating is lustrous and metallic in appearance and provides the steel substrate with exceptional 60 protection against corrosion. Besides the exceptional corrosion protection, the oxidized coating is still extremely thin by prior art standards, being from 1.0 to 5.0 microinches in thickness and weighing no more than 85 mg. per square foot.

If the porous and discontinuous coating is cooled in the 65 vacuum and then subsequently oxidized by prior art practices,

i.e., reheating the coated steel from room temperature in an oxidizing atmosphere, surface oxidation does occur, but it is not nearly as effective in corrosion protection or resistance to discoloration, even if oxidizing temperatures in excess of 600° F. are eventually reached. Hence, the superior product of this invention can be achieved only if high-temperature oxidation, i.e., 600° to 1,000° F., is effected with the substantial exclusion of high-temperature oxidation below 600° F.

We refer to the undesired oxidation as "high-temperature oxidation below 600° F.," because we have learned that a modest degree of room temperature oxidation is not particularly harmful, probably because it is not very extensive. Specifically, coated but unoxidized steels have been cooled to room temperature in the vacuum and then stored in air for periods of about a week or more. These samples, when reheated in a high vacuum to temperatures within the essential oxidizing range, i.e., 600° to 1,000° F., and then quickly exposed to air, did yield the superior protective coating of this invention. On the other hand, samples first exposed to high-temperature oxidation below 600° F. were substantially inferior and could not be improved by further oxidation at temperatures exceeding 600° F. It is apparent therefore that the improved coating of this invention can be achieved only if substantially all oxidation is effected quickly at temperatures within the range 600° to 1,000° F., and that any preliminary oxidation at temperatures below 600° F. down to about 200° F. should be positively avoided.

Although we do not completely understand the mechanism of this invention, we do believe the superior characteristics of our coating results from the combination of the two essential requirements, i.e., the high-purity nature of the chromium coating and the high-temperature oxidation of exposed steel at pores and cracks to form iron oxide magnetite. More specifically, the high-temperature oxidation of this invention causes the pores and cracks in the chromium coating to be plugged with the impervious iron oxide magnetite,  $Fe_3O_4$ . In contrast, lower temperature oxidation typical of the prior art will result in the formation of a more porous oxide,  $Fe_2O_3$ . The magnetite obviously provides superior corrosion protection. Subsequently, when the oxidized coating is cooled, the high-purity nature of the chromium coating contributes ductility thereto, and hence resists cracking that might otherwise occur at temperatures below 600° F. Hence, the finished product coating contains only the original cracks and pores which are plugged with the impervious magnetite. On the other hand, if the chromium coating should contain more typical impurities, particularly iron oxides at the interface, the chromium coating will be more brittle and will crack upon cooling. The new cracks will then be plugged with the more porous  $Fe_2O_3$  formed at temperatures below 600° F.

The chromium coating produced in accordance with this invention is substantially cleaner and of higher purity than most

deposition at temperatures exceeding 500° F. prevents absorption of residual gases on the steel surface where they could react with the deposited chromium. In addition, the deposition pressure, using no greater than  $4 \times 10^{-4}$  torr, reduces the amount of gas reacting with, or occluded in, the chromium coating as it is deposited. Upon the subsequent high-temperature oxidation, the outer surface of the chromium coating is oxidized to some degree, but not sufficient to alter the more ductile characteristics of the chromium beneath the outer oxide skin.

To aid in a fuller understanding of this invention, the following detailed example exemplifies one procedure that may be followed in the practice of this invention.

15

#### EXAMPLE 1

A steel substrate panel (6×4 inches) was cathodically cleaned in a 6 percent solution of Oakite Rustrripper (a proprietary chelating alkaline cleaner) at about 180° F. for 10 seconds at 100 amperes per square foot (a.s.f.), rinsed in tap water, pickled 3 seconds in a 5 percent citric acid solution at about 130° F. or for 1 second at 150° F., rinsed with methanol, warm air dried and placed in the vacuum chamber. The chamber was evacuated to about  $5 \times 10^{-5}$  torr, the substrate was heated to 800° F., a measured quantity of chromium was evaporated and condensed on the substrate with a coating weight of 17 mg./sq. ft., and the vacuum chamber was immediately opened to the air and reached atmospheric pressure in less than 10 seconds. The coated panel was then tested.

30

#### EXAMPLE 2

A steel panel was cathodically cleaned in 1.5 percent Pennsalt 78 cleaner (a proprietary alkaline cleaner) at about 185° F. for 10 seconds at 65 a.s.f., rinsed in water, pickled 30 seconds in 5 percent citric acid at room temperature, rinsed in fresh citric acid solution, rinsed cathodically for 1 second at about 10 a.s.f. in a solution containing approximately 2 percent sodium dichromate with 0.2 percent chromic acid, rinsed in water, warm air dried, and placed in the vacuum chamber. The chamber was evacuated to less than  $10^{-4}$  torr, the substrate was heated to 1,000° F., nichrome (80 percent nickel—20 percent chromium) was evaporated and condensed on the substrate to reach a coating weight of about 34 mg./sq. ft., and oxygen was rapidly admitted to the vacuum chamber to 1 atmosphere pressure. The coated panel was then tested.

40

45

#### EXAMPLE 3

A steel substrate panel was cathodically cleaned at approximately 100 a.s.f. at 180° to 190° F. for 1 minute in a 6 percent solution of Oakite Super Rustrripper (a proprietary chelated alkaline cleaner), rinsed with a water solution containing Par-

From table I it can readily be seen that the resulting corro-

TABLE I.—VACUUM-DEPOSITED-CHROMIUM COATED STEEL HUMID-STORAGE RUST RESISTANCE

| Substrate temperature during coating deposition, ° F. | Specimen temperature during oxidation in air, ° F. | Coating thickness, microinches | Rust resistance in storage at 100° F., 85% relative humidity |            |                          |
|-------------------------------------------------------|----------------------------------------------------|--------------------------------|--------------------------------------------------------------|------------|--------------------------|
|                                                       |                                                    |                                | At 8 days                                                    | At 19 days | Time to 30% rusted, days |
| 800                                                   | 200                                                | 0.5                            | 20                                                           | 90         | ca. 8                    |
| 800                                                   | 400                                                | 0.5                            | 30                                                           | 90         | ca. 8                    |
| 800                                                   | 600                                                | 0.5                            | 30                                                           | 30         | ca. 8                    |
| 800                                                   | 800                                                | 0.5                            | 0                                                            | 10         | 50                       |
| 400                                                   | 200                                                | 0.5                            | 50                                                           | -----      | <8                       |
| 400                                                   | 400                                                | 0.5                            | 60                                                           | -----      | <8                       |
| 400                                                   | 600                                                | 0.5                            | 40                                                           | 60         | ca. 8                    |
| 400                                                   | 800                                                | 0.5                            | 10                                                           | 30         | 19                       |
| 800                                                   | 200                                                | 2.0                            | 0                                                            | 40         | <19                      |
| 800                                                   | 400                                                | 2.0                            | 0                                                            | 30         | 19                       |
| 800                                                   | 600                                                | 2.0                            | 10                                                           | 10         | 50                       |
| 800                                                   | 800                                                | 2.0                            | 0                                                            | 0          | >61                      |
| 400                                                   | 200                                                | 2.0                            | 40                                                           | 90         | <8                       |
| 400                                                   | 400                                                | 2.0                            | 80                                                           | -----      | <8                       |
| 400                                                   | 600                                                | 2.0                            | 40                                                           | 60         | <8                       |
| 400                                                   | 800                                                | 2.0                            | 0                                                            | 20         | ~25                      |

prior art coatings because of the extensive cleaning of the substrate steel surface prior to deposition. Furthermore, vacuum

sion resistance severely drops off as oxidation temperature is reduced.

kin Chemical Company Rust Preventative Additive, warm air dried, and placed in the vacuum chamber. The chamber was evacuated to about  $5 \times 10^{-5}$  torr, the substrate was heated to 600° F., chromium was evaporated from a zirconium-chromium alloy to achieve a coating weight of about 85 mg./sq. ft., the vacuum chamber was quickly opened to a humid air atmosphere, and the panel was removed for testing.

To further exemplify the characteristics of this invention, table I below shows 16 typical experimental samples of steel vapor deposited with chromium and oxidized using various parameters. Both parameters within and outside of the scope of this invention are shown for the purpose of exemplifying the importance of high-temperature oxidation.

Table II below contrasts the corrosion-resistance characteristics (Double Seam Rust Test) of five typical experimental samples processed in accordance with this invention with commercial samples of prior art tin-free steels.

TABLE II.—VACUUM-DEPOSITED-CHROMIUM COATED STEEL CONTRASTED TO COMMERCIAL PRIOR ART TIN-FREE STEEL IN DOUBLE SEAM RUST TEST<sup>1</sup>

| Product tested                        | Coating thickness, microinches | Temperature of deposition of coating, °F. <sup>2</sup> | Rusting on cover hook radius, percent |       |
|---------------------------------------|--------------------------------|--------------------------------------------------------|---------------------------------------|-------|
|                                       |                                |                                                        | Average                               | Range |
| Vac. dep. Cr.                         | 0.5                            | 500                                                    | 15                                    | 9-20  |
| Do                                    | 0.5                            | 800                                                    | 6                                     | 5-8   |
| Do                                    | 2.0                            | 600                                                    | 5                                     | 3-8   |
| Do                                    | 2.0                            | 800                                                    | 6                                     | 2-13  |
| Do                                    | 2.0                            | 800                                                    | 4                                     | 2-6   |
| Prior Art Tin-Free Steel <sup>3</sup> | ~0.5                           | <200                                                   | 41                                    | 35-53 |
| Do                                    | ~0.5                           | <200                                                   | 34                                    | 18-54 |
| Do                                    | ~0.5                           | <200                                                   | 56                                    | 28-99 |
| Do <sup>4</sup>                       | 1.5                            | <200                                                   | 21                                    | 16-44 |
| Do                                    | 1.5                            | <200                                                   | 26                                    | 6-36  |
| Do                                    | 1.5                            | <200                                                   | 18                                    | 6-31  |
| Do <sup>4</sup>                       | ~0.5                           | <200                                                   | 27                                    | 11-62 |
| Do                                    | ~0.5                           | <200                                                   | 43                                    | 24-89 |

<sup>1</sup> Double Seam Rust test simulates rusting which can occur on edge of can end during pasteurization or food processing. Electroplated TFS-CT has rarely done well in this test.

<sup>2</sup> Electroplated TFS-CT coatings cannot be applied at temperatures over the boiling point of the aqueous solutions from which they are deposited. In practice, temperatures are well under 200° F.

<sup>3</sup> Chromium-chromium oxide coating, commercially produced by a one step process.

<sup>4</sup> Phosphate-chromate coating.

<sup>5</sup> Chromium-chromium oxide coating, commercially produced by a two step process.

Our extensive testing and experimentation revealed that the benefits of this invention could not be realized on electrodeposited chromium surfaces. In fact, heating of electrodeposited surfaces in an oxidizing environment actually reduced their corrosion resistance and caused some discoloration.

It should be apparent that various modifications and alternative procedures could be incorporated into the above detailed procedure without departing from the basic concept of this invention. For example, the steel substrate need not be a sheet product intended as a substitute for tinplate. Any cleaning procedure for cleaning the surface of the substrate may be suitable if it is effective in removing substantially all surface scale and oil. In addition, it should be apparent that one of the prime requirements is that the steel, once vacuum-deposited with metallic chromium, not be subjected to low-temperature oxidation. Therefore, the freshly deposited chromium coating need not be oxidized as described immediately after deposition, provided there is no high-temperature oxidation below 600° F.

We claim:

1. A method of producing a corrosion-resistant steel by depositing a protective oxide coating thereon, the steps comprising:
  - a. cleaning the surface of the steel substrate to remove substantially all scale and oils;
  - b. heating the cleaned steel to a temperature of from 500° to

1,000° F. while said steel is subjected to a vacuum of less than about  $4 \times 10^{-4}$  torr;

c. vacuum-depositing metallic chromium onto the heated steel surface to provide a chromium layer of at least about 0.2 microinches;

d. avoiding any substantial oxidation at temperatures between 200° and 600° F. until after step (e);

e. exposing the chromium coated steel to an oxidizing atmosphere while said steel is at a temperature of from 600° to 1,000° F. to form  $Fe_3O_4$  over the steel surfaces exposed through the chromium coating; and

f. cooling said coated steel.

2. The method of claim 1 in which said chromium layer is vacuum-deposited to a thickness of from 0.2 to 20 microinches.

3. The method of claim 1 in which said chromium layer is vacuum-deposited to a thickness of from 1 to 5 microinches.

4. The method of claim 1 in which said vacuum is less than about  $1 \times 10^{-4}$  torr.

5. The method of claim 1 in which said vacuum deposition of chromium is effected at a temperature of from 600° to 800° F.

6. The method of claim 1 in which said chromium coated steel is exposed to said oxidizing atmosphere immediately after the vacuum deposition.

7. The method of claim 1 further comprising the steps of cooling the chromium coated steel to temperatures below about 200° F. in said vacuum after the vacuum deposition of chromium, storing the cooled coated steel in air for periods no greater than about 1 week, reheating the coated steel in a vacuum of less than about  $4 \times 10^{-4}$  torr to a temperature of from 600° to 1,000° F., exposing the reheated coated steel to an oxidizing atmosphere, and then cooling the coated steel.

8. A steel having a corrosion-resistant protective coating consisting of a substantially oxygen free steel substrate having a high-purity vacuum-deposited chromium coating of at least 0.2 microinches in thickness, all pores, cracks and discontinuities in said chromium coating being plugged with a dense, non-porous magnetite.

9. The steel of claim 8 in which said chromium coating has a thickness of from 0.2 to 20 microinches.

10. The steel of claim 8 in which said chromium coating has a thickness of from 1 to 5 microinches.

\* \* \* \* \*

UNITED STATES PATENT OFFICE  
CERTIFICATE OF CORRECTION

Patent No. 3,634,147 Dated January 11, 1972

Inventor(s) Lawrence E. Helwig et al

It is certified that error appears in the above-identified patent and that said Letters Patent are hereby corrected as shown below:

Column 2, lines 31 and 32, cancel "and preferably less than  $1 \times 10^{-4}$  torr" and insert a period (.); line 47, "some what" should read -- somewhat --. Column 4, the paragraph placed immediately before and continued after "Table 1" should be inserted in column 5, between lines 13 and 14.

Signed and sealed this 7th day of November 1972.

(SEAL)

Attest:

EDWARD M. FLETCHER, JR.  
Attesting Officer

ROBERT GOTTSCHALK  
Commissioner of Patents